

# United States Patent [19]

Brusakov et al.

[11] 3,775,092

[45] Nov. 27, 1973

[54] **METHOD OF REFINING  
ALUMINIUM-SILICON ALLOYS**

[76] Inventors: **Jury Ivanovich Brusakov**, Novo-Izmailovsky prospekt, 37, kv. 42; **Irma Solomonovna Livshits**, 3 linia, 48, kv. 21; **Vasily Pavlovich Kiselev**, ulitsa Lensoveta, 48, kv. 10; **Vasily Mikhailovich Cheltsov**, prospekt Kosmonavtov, 38, korpus 2, kv. 92, all of Leningrad; **Mikhail Pavlovich Avdeev**, 7 kvartal, 30, kv. 7, Shelekhov, Irkutskoi oblasti; **Semen Panteleevich Marin**, ulitsa 40 let Sovetskoi Ukrayny, 86, kv. 53, Zaporozhie; **Miro Khristoforovich Alivovodich**, ulitsa 40 let Sovetskoi Ukrayny, 46, kv. 21, Zaporozhie; **Alexei Kuzmich Kulikov**, ulitsa 40 let Sovetskoi Ukrayny, 66, kv. 76, Zaporozhie; **Ivan Arkhipovich Berezhnoi**, ulitsa Patrioticeskaya, 15, kv. 20, Zaporozhie; **Pavel Ilich Volpin**, prospekt Lenina, 210, kv. 16, Zaporozhie; **Leonid Vladimirovich Chernyakhovsky**, ulitsa Kizhne-Dneprovskaya, 4b, kv. 75, Zaporozhie; **Zoya Vasiliyevna Eltsova**, ulitsa 40 let Sovetskoi Ukrayny, 6, kv. 71, Zaporozhie; **Lidia Nikolaevna Medvedeva**, ulitsa 40 let Sovetskoi Ukrayny, 66, kv. 172, Zaporozhie; **Fedor Mifodievich Kolomitsky**, ulitsa 21 Partsiezda, 16, kv. 92, Zaporozhie, all of U.S.S.R.

[22] Filed: Aug. 24, 1971

[21] Appl. No.: 174,533

[30] **Foreign Application Priority Data**

Nov. 11, 1970 U.S.S.R. .... 1485657  
Nov. 11, 1970 U.S.S.R. .... 1485664

[52] U.S. Cl. .... 75/68 A, 75/93 AC  
[51] Int. Cl. .... C22b 21/06  
[58] **Field of Search** .... 75/68 A, 93 AC

[56] **References Cited**

UNITED STATES PATENTS

2,184,705 12/1939 Willmore .... 75/68 A  
2,255,549 9/1941 Kruh .... 75/68 A  
380,577 9/1932 Lightalloy Ltd. .... 75/68 R

FOREIGN PATENTS OR APPLICATIONS

964,792 7/1964 Great Britain .... 75/68 A

OTHER PUBLICATIONS

Handbook of Chemistry and Physics; Chemical Rubber Co.; 50th Edition; 1969; page B-157.

*Primary Examiner*—L. Dewayne Rutledge

*Assistant Examiner*—M. J. Andrews

*Attorney*—Holman & Stern

[57] **ABSTRACT**

The method consists in that the aluminum-silicon alloy is first treated with flux at a temperature not under 1,500°C, then it is treated with more of the same flux at 900°-1,200°C.

**3 Claims, No Drawings**

## METHOD OF REFINING ALUMINIUM-SILICON ALLOYS

The present invention relates to refining aluminium-silicon alloys produced in ore-reduction furnaces in order to remove nonmetallic admixtures from them.

According to the present invention a flux with a fluorosilicic constituent is provided which is useful in refining the diluted aluminium-silicon or other structural aluminium alloys.

Methods are known in the art for refining aluminium-silicon alloys containing more than 30 percent Si by removing non-metallic inclusions from them with the aid of a flux consisting of a mixture of chlorides and fluorides of alkali and/or alkaline-earth metals with preliminary cooling of the alloy down to 900°C or down to 1,100°-1,300°C.

A method is also known in the art for refining casting aluminium-silicon alloys with the aid of a number of general-purpose fluxes consisting of chlorides and fluorides of alkali and/or alkaline-earth metals.

However, in the known method, when the alloy is preliminarily cooled to 900°-1,200°C the bulk of the nonmetallic inclusions, functioning as additional nuclei of crystallization, settles on the walls and bottom of the ladle together with silicon (beginning with 1,100°C) entraining the metal and thus increasing its losses. At these temperatures the alloy features a higher viscosity and the process of its refining is comparatively slow. The known methods are adapted only for fine refining of the alloy from a small quantity of admixtures.

The fluxes are used in refining the aluminium-silicon alloys not only for removing the nonmetallic admixtures from the alloy, but also for protecting the alloy surface against oxidation. With this purpose in view the flux melting point should be equal to, or somewhat lower than, the temperature at which the alloy is processed. However, the melting point of the known fluxes used for refining the casting aluminium-silicon alloys is 130°-200°C higher than the required temperatures which prevents complete protection of the alloy against oxidation, thus increasing the losses of alloy.

Besides, these fluxes contain a considerable proportion of cryolite or sodium fluoride which raise the cost of the flux.

The main object of the invention resides in selecting the optimum conditions under which the alloy would be best refined from nonmetallic inclusions.

This and other objects are accomplished by the use of a method of refining aluminium-silicon alloys produced in ore-reduction electric furnaces by introducing a flux containing fluorides and chlorides of alkaline and/or alkaline-earth metals at a temperature of 900°-1,200°C wherein, according to the invention, the alloy is first mixed with a flux at a temperature of not under 1,500°C.

For better protection of the surface of the aluminium-silicon alloy against oxidation, it is practicable to use a flux containing the fluosilicate of alkaline metals and having the following composition (per cent):

fluosilicate of alkali metals — 38-40

sodium chloride — 45-47

potassium chloride — 14-16

Now the invention will be described in detail by way of examples.

The claimed method of refining aluminium-silicon alloys includes the following operations: as the ladle is

being gradually filled with the primary alloy from the furnace tap hole, said alloy is mixed with 2-4 percent of flux (from the total weight of the alloy), said flux consisting of a mixture of chlorides and fluorides of alkali and/or alkaline-earth metals. The alloy temperature in the ladle should not be lower than 1,500°C. The flux introduced at such a temperature is conducive to coagulation of nonmetallic admixtures, thereby reducing the viscosity of the alloy. The aluminium-silicon alloy 5 preliminarily treated with fluxes is again refined at 900°-1,200°C, the quantity of the flux being 4-6 percent of the total weight of the alloy.

The alloy pretreated by preliminary refining has a lower viscosity so that refining is sufficiently complete 10 and the losses of the alloy, particularly of silicon, are reduced.

The flux according to the invention wherein the fluoride component is replaced by fluosilicate improves the protection of the alloy surface against oxidation at the 15 same time retaining the adequate degree of refining the alloy from nonmetallic inclusions.

Besides, said fluosilicate component is markedly 20 cheaper (three times approximately) than the fluoride component (cryolite, sodium fluoride, etc.).

It is most practicable to use for these purposes a flux 25 having the following composition (per cent):

fluosilicic component of alkali metals — 38-40  
sodium chloride — 45-47  
potassium chloride — 14-16

30 The fluosilicic component may be either sodium fluosilicate or potassium fluosilicate.

Now the invention will be made more apparent by 35 describing the examples of its realization.

### EXAMPLE 1

Let us consider two cases of refining a primary aluminium-silicon alloy. In both cases the alloy is refined at a temperature of 1,200°-1,300°C. Besides, in the first case the alloy is preliminarily refined at a temperature of 1,600°C while in the other case the alloy is not refined at high temperatures. High-temperature refining (1,600°C) produces 670 kg of refined alloy from 1,000 kg of primary alloy.

When the alloys are refined without high- 40 temperature treatment with fluxes, only 635 kg of refined alloy are obtained from 1,000 kg primary alloy which means that the alloy losses are increased.

The yield of the alloy owing to additional refining at a temperature of 1,600°C increases as much as 5.5 percent.

### EXAMPLE 2

Tests at 1,500°C have been made of the flux with the following composition:

55 potassium fluosilicate — 38.64 percent  
sodium chloride — 46.21 percent  
potassium chloride — 15.09 percent

The aluminium-silicon alloy was mixed with the flux of the above-stated composition in the quantity of 2 60 percent of the total weight of the alloy.

A comparison of the results of refining obtained by the use of the known and claimed fluxes has shown that the yield of the refined alloy has remained the same though the quality of the refined alloy with respect to the nonmetallic inclusions, as determined by a metallographic analysis has proved to be considerably higher.

| alloy | alloy | Yield | Flux composition                 |       |       |
|-------|-------|-------|----------------------------------|-------|-------|
| tons  | tons  |       | K <sub>2</sub> SiF <sub>6</sub>  | NaCl  | KCl   |
| 300.0 | 272.3 | 90.7  | 38.64                            | 46.21 | 15.09 |
| 300.0 | 270.5 | 90.2  | Na <sub>3</sub> AlF <sub>6</sub> | NaCl  | KCl   |
|       |       |       | 20.0                             | 40.0  | 40.0  |

Besides, the flux with a fluosilicic component cuts down the prime cost of the final product, i.e., silumin or other structural alloys.

On the basis of this invention we hereby claim a method of refining the aluminium-silicon alloy which ensures a more efficient refining of the alloy from non-metallic inclusions which, during further treatment of the alloy, leads to a higher yield of the marketable product. The use of the flux with the above-stated composition reduces the percentage of nonmetallic inclusions in the refined alloy; besides, the cheaper flux re-

duces the prime cost of the alloy.

What is claimed is:

1. A method of refining aluminum-silicon alloys produced in ore-reduction electric furnaces comprising introducing into said alloy at a temperature of not under 1,500°C a first portion of a flux containing the fluorides and chlorides of alkali and alkaline-earth metals and adding a second portion of said flux to the alloy at a temperature of 900°-1,200°C.

2. A method according to claim 1, wherein said first portion of said flux is about 2-4 percent by weight of the alloy.

3. A method according to claim 1, wherein the total quantity of said flux is about 4-6 percent by weight of the alloy.

\* \* \* \* \*

20

25

30

35

40

45

50

55

60

65